

## UNITED STATES PATENT OFFICE

2,488,246

PROCESS OF ELECTROPLATING ZINC AND  
BATHS AND COMPOSITIONS FOR USE  
THEREIN

Jesse E. Stareck, Birmingham, and Frank Pas-  
salacqua, Detroit, Mich., assignors to United  
Chromium, Incorporated, New York, N. Y., a  
corporation of Delaware

No Drawing. Application August 25, 1944,  
Serial No. 551,258

4 Claims. (Cl. 204—55)

1

This invention relates to the electrodeposition of zinc, and provides improvements therein.

The invention provides a new and improved process for electrodepositing zinc, and novel baths and compositions for use in such process.

It is desirable and advantageous (1) to electroplate smooth zinc deposits, (2) to electroplate bright deposits of zinc, (3) to electroplate such deposits with high current efficiency, (4) to make use of noncyanide alkaline baths which are free from cyanide fumes, (5) to make use of baths less alkaline than cyanide-zinc baths, yet of such alkalinity that iron is not soluble in the bath, (6) to have baths in which the pH remains fairly stable, (7) to have an alkaline bath with which air or mechanical agitation can be used without building up carbonates or other objectionable reaction products therein, (8) to electrodeposit zinc at greater speed than by other processes making use of alkaline baths, (9) to avoid as much as possible hydrogen embrittlement of the base metal in the process of electrodepositing the zinc, (10) to obtain brighter deposits than are obtained by processes heretofore used, (11) to electrodeposit zinc on cast iron without special preliminary steps, (12) to have a process of electrodepositing zinc which works well in barrel plating, (13) to make use of baths which are not corrosive to equipment and which do not give off poisonous fumes; the foregoing advantages are obtained by the use of the process and baths of the present invention.

According to the present invention a bath is used which contains the complex compound potassium zinc pyrophosphate  $K_6Zn(P_2O_7)_2$ , having a controlled pH, and containing a substance which acts as a brightener and a throwing power promotor. The pyrophosphate radicals and zinc content are in the molecular ratio of 2 to 1 plus an excess of pyrophosphate radicals; with said excess the molecular weight ratio range is from 2.3 to 1 to 4.6 to 1.

Compositions of water soluble zinc and pyrophosphate compounds may be made up for preparing baths with zinc and pyrophosphate radical contents as given above.

The bath may contain other substances which give known effects, such as wetting agents, anti-foamants, buffering agents, anode depolarizers, etc.

For making up the bath, (and also the composition of matter) a zinc compound such as zinc sulphate or zinc chloride or zinc pyrophosphate soluble in an aqueous solution of potassium or sodium pyrophosphate, and potassium or sodium pyrophosphate, may be used. The sodium pyrophosphate is less soluble than the potassium pyrophosphate. As the commercial chemicals vary somewhat in composition, they should be

used on the basis of the ascertained pyrophosphate and zinc content.

## Examples of baths

G./1.

|     |                          |     |
|-----|--------------------------|-----|
| I.  | $Zn_2P_2O_7 \cdot 3H_2O$ | 68  |
|     | $K_4P_2O_7$              | 360 |
|     | corresponding to         |     |
|     | $Zn$                     | 25  |
|     | $P_2O_7$                 | 225 |
| II. | $ZnSO_4 \cdot 7H_2O$     | 110 |
|     | $K_4P_2O_7$              | 375 |
|     | corresponding to         |     |
|     | $Zn$                     | 25  |
|     | $P_2O_7$                 | 225 |

The concentrations of the bath constituents can be greater or less than those given in the examples above; the concentrations given are good working concentrations.

A brightener is added to the bath, and is a solution soluble carbocyclic compound having hydroxy and methoxy groups ortho to one another, specific examples of which are curcumin, phenol sulphonate condensation products of vanillin, and ortho-hydroxy meta-methoxy benzaldehyde, the last of which we have found to be the most satisfactory to use. Vanillin is also included in the above class, its usefulness, however, appearing to be in baths having a pH of about 9.5. Brighteners of this type, when added to the bath, act as very efficient hydrogen inhibitors during plating, especially on ferrous base metals. Besides producing a brightening action, the addition of brighteners will also markedly increase the operating current density range. Oxidation products of the brightener, as produced by electrolysis or the addition of an oxidizing agent as for example potassium permanganate, act as promoters of throwing power.

The quantity of brightener used is small as regards the other bath constituents, and in the baths according to the examples given above, the concentration is generally maintained at one-half to three grams per liter depending on the brightener used and its solubility. The brightener should be added to the bath in amounts to produce brightness under optimum working conditions. The brightness of the zinc deposit equals that of mirror-like chromium deposits with which the art is familiar.

The alkalinity, or pH, of the bath is maintained between 9.5 and 12.5, with the optimum between 11.2 and 12.0. The effect of maintaining the bath in the aforesaid pH range is to eliminate roughness of the deposit and to give complete coverage, with the brightener present; high current efficiencies are also obtained. It is an important and concomitant advantage of the invention that the range of pH or alkalinity of

the bath is above the pH value at which iron dissolves in the bath. Potassium hydroxide may be used to raise the pH and pyrophosphoric acid to lower it. The pH of baths according to the present invention remain stable in operation, which is an advantage of the invention.

Bath temperature may vary over a considerable range; for reasonable speed of deposition and brightness of the zinc deposit, temperatures from room temperature to 140° F. may be used.

The average current density may also vary considerably; with baths of the composition given in the above examples, current densities up to 80 amperes per square foot may be used with good results. With the aforesaid baths, current densities of 20 to 70 amperes per square foot are optimum. The current efficiency is nearly 100%, and the process of the present invention, over other alkaline processes for electrodepositing zinc, has the advantage of causing much less hydrogen embrittlement. Moreover, the speed of deposition is considerably higher than with other alkaline baths heretofore in use. The throwing power is good, being better than that of acid-zinc processes, and generally better than that obtained from cyanide-zinc processes.

It is desirable to agitate the baths in operation, and this may be done either by air or mechanical means. Neither carbonates nor other objectionable reaction products accumulate by air agitation. If foaming occurs this can be eliminated by means of adding a suitable antifoaming agent. We have discovered a novel and very advantageous antifoaming agent for use in our baths in the substance tri-octylphosphate.

For anodes, electrolytic zinc or cast zinc of high purity is recommended. Citrate radical in the bath, in quantity of about 15 g./l., may be used as a depolarizer.

Care should be taken to exclude metallic impurities, especially lead, hexavalent chromium, copper, cadmium and arsenic. In general, the bath should be kept pure.

It is desirable to electrolyze the baths before using for plating operations, or to add a small quantity of potassium permanganate to build up or promote the throwing power of the bath.

A mode of procedure followed in the plating of steel cartridge cases is as follows:

*Bath composition*

|                                                      |       |      |
|------------------------------------------------------|-------|------|
| Zn                                                   | g./l. | 23   |
| P <sub>2</sub> O <sub>7</sub>                        | g./l. | 210  |
| Citrate                                              | g./l. | 15   |
| Brightener (ortho hydroxy meta methoxy benzaldehyde) | g./l. | 1    |
| Wetting agent (penta octyl sodium tri polyphosphate) | g./l. | 1/2  |
| Antifoamant (tri octyl phosphate)                    | g./l. | 0.01 |
| pH                                                   |       | 11.5 |

The steel cartridge cases were put on a rack, immersed in the bath, and connected to the cathode bus-bar. Current was passed for three minutes at a current density of 60 amperes per square foot, at the end of which time there was obtained a uniform, smooth, mirror-bright deposit 0.0002 inch thick. The temperature of the bath was 115° F. and air agitation was used. The anodes were cast electrolytic zinc.

The baths and process of this invention can be satisfactorily used for barrel-plating.

The zinc deposits obtained by the use of the

present invention are smooth, and smooth and bright under optimum operating conditions, the brightness being like that of mirror-like chromium deposits. The deposits have a fine grained crystalline structure typical of truly bright metallic deposits.

What is claimed is:

1. An aqueous bath for electroplating zinc, consisting essentially of pyrophosphate radicals and zinc in the molecular ratio of approximately 2.3 to 1 to 4.6 to 1, and optimum amounts of approximately 1/2 to 3 g./l. of ortho-hydroxy meta methoxy benzaldehyde, acting as a brightener, and having a pH between 9.5 and 12.5.
- 10 2. An aqueous bath for electroplating zinc, according to claim 1, wherein the pH is between 11.2 and 12.0.
- 20 3. A process of electrodepositing smooth zinc plate, which comprises passing an electric current from an outside source from an anode to a cathode-article immersed in an aqueous bath solution at room temperature to 140° F. and at 1 to 80 amperes per square foot consisting essentially of pyrophosphate radicals and zinc in the molecular ratio of approximately 2.3 to 1 to 4.6 to 1, and optimum amounts of approximately 1/2 to 3 grams per liter of ortho-hydroxy meta methoxy benzaldehyde, acting as a brightener, and having a pH between 9.5 and 12.5.
- 25 4. A composition of matter, consisting essentially of an alkali-metal pyrophosphate, zinc pyrophosphate which is soluble in a water solution of the alkali-metal pyrophosphate, and ortho-hydroxy meta methoxy benzaldehyde as a brightener, the ratio of the pyrophosphate radicals to the zinc in the aforesaid ingredients being in the molecular weight ratio range 2.3 to 1 to 4.6 to 1, and the amount of the brightener being 1/2 to 3 parts brightener for 250 parts zinc and 40 pyrophosphate radicals in the composition.

JESSE E. STARECK.  
FRANK PASSALACQUA.

REFERENCES CITED

- 45 The following references are of record in the file of this patent:

UNITED STATES PATENTS

| Number       | Name         | Date          |
|--------------|--------------|---------------|
| 50 744,170   | Darlay       | Nov. 17, 1903 |
| 809,492      | Classen      | Jan. 9, 1906  |
| 1,681,509    | Westbrook    | Aug. 21, 1928 |
| 1,791,082    | Bianco       | Feb. 3, 1931  |
| 2,080,479    | Hoff         | May 18, 1937  |
| 55 2,250,556 | Stareck      | July 29, 1941 |
| 2,315,607    | Ferm et al.  | Apr. 6, 1943  |
| 2,318,592    | Cupery       | May 11, 1943  |
| 2,360,135    | Hull         | Oct. 10, 1944 |
| 2,393,517    | Burns        | Jan. 22, 1946 |
| 60 2,447,297 | Wegst et al. | Aug. 17, 1948 |

OTHER REFERENCES

- Ser. No. 355,522, Howaldt et al. (A. P. C.) pub. May 18, 1943.
- 65 Journal of American Chemical Society (18) 654.
- Electrodeposition of Metals, by Langbein and Braunt, 9th edition, 1924, page 567.
- Wood Chemistry, by Wise, 1944 edition, pages 70 272-360.
- Transactions of the Electrochemical Society, vol. 88 (1945), page 272.